

## UNITED STATES PATENT OFFICE

KENNETH G. MACKENZIE, OF WESTPORT, CONNECTICUT, ASSIGNOR TO THE TEXAS COMPANY, OF NEW YORK, N. Y., A CORPORATION OF DELAWARE

## LUBRICATING OIL

No Drawing.

Application filed July 12, 1930. Serial No. 467,628.

This invention relates to lubricating oils and more particularly to lubricating oils which are compounded, having hydrocarbon oils or derivatives thereof as a base.

5 Considerable work has been done of late by certain investigators in connection with the manufacture and use of extremely low viscosity oils for the lubrication of bearings of electric motors, such as electric railway 10 motors, axle bearings, journal bearings, and other similar or related structures. It has been definitely determined that oils having viscosities as low as 37 seconds at 100° F., and possibly lower, when properly compounded, provide adequate lubrication for 15 the bearing surfaces, and decrease to a marked degree the power consumption costs by reducing the frictional resistance to be overcome upon starting the motor or journal 20 and during the operation thereof.

These low viscosity oils must, however, have certain properties or characteristics to adapt them to the service for which they are intended. The viscosities of the oils 25 should be as low as possible, consistent with flash point for the conditions under which they are to be used. The oils must be sufficiently adherent to remain on the surfaces of the metals under severe conditions of 30 service, and must have sufficient body to act as cushions between the metallic surfaces, even when the parts are at rest. Furthermore, the oils must have that property known as oiliness.

35 These properties have been secured in high degree by compounding an oil or other liquid of the lowest possible viscosity with another substance having high adhesive or adherent properties, such as lard oil, in the 40 proportion of 10% lard oil to 90% of the low viscosity oil or other liquid. It has also been suggested that palm or castor oil, metallic soaps, and oils treated with sulphur or 45 oxygen might in certain cases be utilized.

I have found that a highly desirable product of extremely low viscosity, which has the properties of adhesiveness and extreme oiliness, can be made by compounding with 50 the low viscosity base product, a relatively

small amount of another product which will supply the adhesiveness required to insure constant adherence of the lubricant to the bearing surfaces. Because of the excellent lubricating value of the added product, less 55 of it ordinarily need be added than of the lard oil heretofore used in order to produce equivalent results.

The added product is stable and does not tend to decompose with age in the manner 60 that animal and vegetable oils become rancid and in this respect the added product is superior to lard oil as the compounding agent. Furthermore, the added product is less expensive than any of the animal or vegetable 65 oils proposed by other investigators, and on this account the ultimate cost of the final product can be lowered and thus made available to a larger market.

In United States Patent No. 1,705,298 issued 70 jointly to me and Raymond Haskell on March 12, 1929, we have described a lubricating oil comprising a hydrocarbon oil and oxidized paraffin wax. We found that the addition of a small amount of oxidized 75 paraffin wax to the usual hydrocarbon lubricating oil produced very beneficial effects. The oxidized paraffin wax which is used in compounding our lubricating oil, as described in Patent No. 1,705,298, is produced 80 by blowing crude or refined wax with air at an elevated temperature. A change takes place in the chemical characteristics of the material, acidity developing not only as evidenced by the increasing acidity of the material 85 itself, but also by the fact that some volatile acids may be condensed from the air after it has passed through the hot material.

In addition to these, however, certain saponifiable bodies or esters are formed, apparently from condensation of acids and alcohols produced by the oxidation. These esters are found to differ from the saponifiable oils and fats in that they do not readily 90 saponify when treated with aqueous alkali solution but require treatment with an alcoholic solution of alkali to effect complete saponification.

Upon separation of the constituents of the 100

- oxidized paraffin wax and compounding them separately with hydrocarbon lubricating oil, it is found that the previously mentioned esters, when so used, greatly increase the lubricating properties of a hydrocarbon oil. However, inasmuch as the acids and the unchanged wax in the oxidized material do not adversely effect the valuable properties of the esters, the oxidized wax itself may be used for compounding, thus avoiding the expense involved in the extraction of the esters.
- In ordinary methods of oxidizing paraffin wax the material is heated while exposed to a current of air until practically complete oxidation takes place. The procedure yields a product which usually has very unsatisfactory properties rendering it unsuitable for compounding with mineral oils due to the fact that the high oxidation products are dark colored gummy materials insoluble in hydrocarbon oil. To produce a product suitable for compounding, I depart from the ordinary method and, while carrying the reaction to a fairly definite point as may be evidenced by the acid value of the product, discontinue it before there is any substantial formation of the gumlike products of a more prolonged oxidation. While an acid value of about 40 may be considered the upper limit to which the reaction may be safely carried without the formation of gums, I prefer to only carry the oxidation to an acid value of about 35 which insures the complete absence of gummy constituents.
- At the same time the quantity of unoxidized wax or of little oxidized wax will usually be sufficiently low that the oils compounded with such oxidized wax product will have a low pour test. On the other hand if the amount of little oxidized wax is objectionable from the standpoint of producing compounded oils with too high a pour test for the particular service desired, this may readily be overcome by sweating the oxidized product to any desired degree to remove the higher melting portions thereof.
- The following is a specific example of a method which has been found suitable in the oxidation of paraffin wax to produce a finished product having a sufficiently large proportion of esters. A charge of 50 pounds of paraffin wax is maintained at a temperature of from 295° to 300° F. in an enameled vessel while air is introduced in fine streams at the bottom of the vessel. The rate of introduction of the air is dependent upon the degree of distribution and contact which is obtained with the reaction materials. The oxidation is allowed to proceed for a period of about 48 hours during which time there is a loss of from 7% to 10% in the weight of the charge due to volatilization products being carried off with the air stream.
- A typical sample of material produced by

this treatment has the following characteristics:

|                                                |         |
|------------------------------------------------|---------|
| Acid number                                    | 39.8    |
| Total saponification number                    | 170.5   |
| Neutral saponification number                  | 130.7   |
| Melting point                                  | 107° F. |
| Neutral saponification number<br>(Acid number) | 3.28    |

Another sample of the same material was treated first with alkali to neutralize the free acid and then treated with methyl ethyl ketone in which the paraffin wax is, for practical purposes, insoluble. The following results were obtained:

|                                                                                 | Per cent |
|---------------------------------------------------------------------------------|----------|
| Free acid                                                                       | 22.4     |
| Material insoluble in methyl ethyl ketone (unsaponifiable material, mainly wax) | 16.8     |
| Material soluble in methyl ethyl ketone (saponifiable material, mainly esters)  | 60.8     |

It will be observed from this data that the oxidized wax contains a large amount of saponifiable material and comparatively little unchanged wax.

The aforementioned method of oxidizing paraffin wax is given for the purpose of illustration only, and any other process may be used which will produce an oxidized wax containing a large amount of saponifiable material and comparatively little unchanged wax, as for example, the process described in the patent to J. R. Scanlin No. 1,668,871 dated May 8, 1928.

According to the present invention I prefer to use a lubricating oil stock derived either from petroleum or the products of distillation of coal or shale that has the lowest possible viscosity for the conditions under which the machine operates; that is, the lowest viscosity that is obtainable with the requisite flash point to withstand the temperature prevalent during use.

The lubricating oil stock may consist of an oil having in general the characteristics of kerosene oil, but preferably I prefer to use as stock a product made by distilling off about 75% of the lighter material from kerosene oil and using the remainder in the still as stock for the preparation of the finished lubricant. The flash point should be above 225-230° F. and the viscosity of the stock is preferably within the range of 35 to 45 seconds (Saybolt) at 100° F. The finished product is then compounded with a small proportion of oxidized paraffin wax containing a large amount of saponifiable material and comparatively little unchanged wax. In most instances a compounded product having a viscosity of about 60 seconds or less at 100° F. (Saybolt) and containing from 2%-5% of the wax will give results which are substantially equivalent to those obtained with an oil compounded with about 10% of lard oil, but under some circumstances as

much as 15% of wax may be used, it being understood that the amount of wax may be varied as circumstances may require. Ordinarily, an oil compounded with from 2%—  
 5 3% of oxidized paraffin wax and having a viscosity of 45 seconds or even less at 100° F. (Saybolt) will be satisfactory.

While I have thus specifically described my invention, various modifications thereof  
 10 may suggest themselves to those skilled in the art and I desire therefore to be limited only as indicated in the appended claims.

What I claim is:

1. A lubricating oil for heavy machinery  
 15 consisting of at least 95% of a hydrocarbon oil having a viscosity considerably lower than that normally used for such purposes and within the range of from 37 seconds to 60 seconds (Saybolt) at 100° F. and from 2%  
 20 to 5% of oxidized paraffin wax which has been oxidized in such manner as to contain a large proportion of saponifiable material.

2. A lubricant for railway journals and bearings comprising a mixture of the hydro-  
 25 carbon oil remaining after distilling off about 75% of the lighter constituents of kerosene and having a viscosity within the range of from 37 seconds to 60 seconds (Say-  
 30 bolt) at 100° F. and from 2% to 5% of oxi-  
 dized paraffin wax which has been oxidized in such manner as to contain a large propor-  
 tion of saponifiable material.

3. A lubricant for railway journals and bearings consisting of from 95% to 98% of  
 35 a hydrocarbon oil having a viscosity of ap-  
 proximately 45 seconds (Saybolt) at 100° F. and from 5% to 2% of oxidized paraffin wax which has been oxidized in such manner as to contain a large proportion of saponi-  
 40 fiable material.

In witness whereof I have hereunto set my  
 had this 7th day of July, 1930.

KENNETH G. MACKENZIE.

45

50

55

60